



US005370806A

**United States Patent** [19]

Cardis et al.

[11] **Patent Number:** **5,370,806**[45] **Date of Patent:** **Dec. 6, 1994**[54] **BORATED DIHYDROCARBYL  
DITHiocarbamate Lubricant  
Additives and Composition Thereof**[75] Inventors: **Angeline B. Cardis, Florence;  
Liehpao O. Farng, Lawrenceville;  
Andrew G. Horodysky, Cherry Hill;  
Abraham O. M. Okorodudu, West  
Deptford, all of N.J.**[73] Assignee: **Mobil Oil Corporation, Fairfax, Va.**[21] Appl. No.: **454,537**[22] Filed: **Dec. 21, 1989**[51] Int. Cl.<sup>5</sup> ..... **C10M 139/00; C10M 135/18**[52] U.S. Cl. ..... **252/46.3; 558/236;  
558/286; 558/293; 558/295**[58] Field of Search ..... **558/286, 293, 295, 236;  
252/49.6, 33.6, 47.5, 46.3, 400.4, 400.41; 44/317**[56] **References Cited****U.S. PATENT DOCUMENTS**

|           |         |                    |          |
|-----------|---------|--------------------|----------|
| 2,504,672 | 4/1950  | Farrington et al.  | 252/47.5 |
| 2,673,839 | 11/1954 | Kirshenbaum        | 558/240  |
| 2,756,249 | 7/1956  | Kirshenbaum et al. | 252/47.5 |

|           |         |                 |            |
|-----------|---------|-----------------|------------|
| 3,081,335 | 3/1963  | Morris et al.   | 252/47.5   |
| 3,833,496 | 9/1974  | Malec           | 252/33.6   |
| 4,110,319 | 8/1978  | Lawrence        | 558/240    |
| 4,225,450 | 9/1980  | Rosenberger     | 252/47.5   |
| 4,226,732 | 10/1980 | Reinhard et al. | 252/47.5   |
| 4,360,438 | 11/1982 | Rowan et al.    | 252/47.5   |
| 4,524,005 | 6/1985  | Horodysky       | 558/293    |
| 4,529,529 | 7/1985  | Horodysky       | 558/293    |
| 4,609,480 | 9/1986  | Hata et al.     | 252/47.5   |
| 4,648,985 | 3/1987  | Thorsell        | 252/32.7 E |
| 4,756,842 | 7/1988  | Holstedt        | 252/46.3   |
| 4,759,873 | 7/1988  | Audeh           | 252/49.6   |
| 4,788,340 | 11/1988 | Horodysky       | 252/293    |
| 4,859,353 | 8/1989  | Colclough       | 558/293    |
| 4,997,969 | 3/1991  | Luciani         | 252/47.5   |
| 5,126,063 | 6/1992  | Cardis          | 252/46.3   |

*Primary Examiner*—Margaret Medley*Attorney, Agent, or Firm*—Alexander J. McKillop;  
Malcolm D. Keen; Charles A. Malone

## [57]

**ABSTRACT**

Borated dihydrocarbyl dithiocarbamate reaction products have been found to be effective antioxidant/antiwear multifunctional additives for lubricants.

**20 Claims, No Drawings**

**BORATED DIHYDROCARBYL  
DITHiocarbamate LUBRICANT ADDITIVES  
AND COMPOSITION THEREOF**

**BACKGROUND OF THE INVENTION**

This invention relates to multifunctional antioxidant/antiwear additives and to compositions comprising lubricants, greases and other solid lubricants thereof containing a minor amount of mixed alcohol/dithiocarbamate derived borate.

The metal surfaces of machinery or engines operate under heavy or normal loads wherein the metal is under friction, even when being lubricated. Thus, there is always metal wear which in some cases can be excessive. It is clear that lubricants used to protect the metal surfaces do not completely prevent wear at the points of metal to metal contact. Consequently, the performance of the machine or engine will suffer, and in aggravated cases the machine or engine may become completely inoperative from the wear caused by the friction and the load.

There have been many attempts to devise additive systems to improve the extreme pressure/load carrying properties of a lubricant. The non-metallic derivatives of the present invention provide lubricating oil compositions with enhanced antioxidant/antiwear and extreme pressure/load carrying characteristics and are believed to be capable of overcoming some of the aforementioned deficiencies of prior art additives.

Lubricants, such as lubricating oils and greases, are subject to oxidative deterioration at elevated temperatures or upon prolonged exposure to the elements. Such deterioration is evidenced, in many instances, by an increase in acidity and in viscosity, and when the deterioration is severe enough, it can cause metal parts to corrode. Additionally, severe oxidation leads to a loss of lubrication properties, and in especially severe cases this may cause complete breakdown of the device being lubricated. Many additives have been tried, however, many of them are only marginally effective except at high concentrations. Improved antioxidants are clearly needed.

Antioxidants or oxidation inhibitors are used to minimize the effects of oil deterioration that occur when, for example, hot oil is contacted with air. The degree and rate of oxidation will depend on temperature, air and oil flow rates and, of particular importance, on the presence of metals that may catalytically promote oxidation. Antioxidants generally function by prevention of chain peroxide reaction and/or metal catalyst deactivation. They prevent the formation of acid sludges, darkening of the oil and increases in viscosity due to the formation of polymeric materials.

Water (moisture) is another critical problem. In spite of even extraordinary precautionary efforts water is found as a film or in minute droplets in vessels containing various hydrocarbon distillates. This brings about ideal conditions for corrosion and damage of metal surfaces of the vessels and the materials contained therein. Also in the lubrication of internal combustion engines, for example, quantities of water are often present as a separate phase within the lubricating system. Another serious problem in respect to metallic surfaces in contact with adjacent metallic surfaces is the surface wear caused by the contact of such surfaces. One mate-

rial capable of simultaneously coping with such problems effectively is highly desireous.

The use of metal dithiocarbamates (such as zinc, nickel, or lead dialkyl dithiocarbamates) are known as effective antioxidants and antiozonants for many rubbers and polymers in various kinds of applications, such as SBR and NBR.

The non-metallic (ashless) dithiocarbamates, such as 4,4'-methylene bis(dibutyl dithiocarbamate), have been well known for their antioxidant and extreme pressure properties in lubricant applications.

The use of borate has been widely reported as having beneficial multifunctional friction reducing properties, as well as antioxidant properties in lubricant applications.

It has now been found that the use of these alcohol or hydroxy-hydrocarbyl/dithiocarbamate-derived hydroxy borates provides exceptional antioxidant and antiwear/EP activity with potential antifatigue and high temperature stabilizing properties.

**SUMMARY OF THE INVENTION**

This application is therefore directed to lubricant compositions containing small additive concentrations of mixed alcohol/S-hydroxyalkyl N,N-dihydrocarbyl dithiocarbamate-derived borates which possess excellent antioxidant properties coupled with very good antiwear and extreme pressure load carrying activities. Both the dithiocarbamate moiety and the borate moiety are believed to provide the basis for the synergistic antioxidant activity. The dithiocarbamate group is also believed to contribute significant antiwear property to these novel additives.

All of these beneficial properties are believed to be enhanced as a result of this novel internal synergism. This unique internal synergism concept is believed to be applicable to similar structures containing (a) dithiocarbamate groups, (b) borate groups within the same molecule. The products of this patent information show good stability and compatibility when used in the presence of other commonly used additives in lubricant compositions.

The lubricant compositions described herein are believed to be novel and their use as antioxidant/antiwear and extreme pressure/load carrying lubricant additives is also believed to be novel.

**DESCRIPTION OF SPECIFIC EMBODIMENTS**

Metallic, e.g., sodium dialkyl dithiocarbamates may be synthesized by reacting equal molar amounts of metallic hydroxide such as sodium or potassium hydroxide or the like, a secondary dialkyl amine, and carbon disulfide in aqueous media or organic solution depending on conditions (Equation 1).



Similarly, triethylammonium salts of dithiocarbamates can be made by reacting triethylamine, dialkylamine and carbon disulfide in the non-aqueous media (Equation 2).



This structure is more generally represented as



where  $R_1, R_2$  are  $C_1$  to about  $C_{60}$  hydrocarbyl,  $R_3$  is  $C_1$  to about  $C_{50}$  hydrocarbyl and  $M$  is a metal cation.

Propylene oxide (1,2-epoxypropane) was reacted with either sodium dialkyl dithiocarbamates or triethylammonium salts of dialkyl dithiocarbamates to form S-hydroxypropyl N,N-dialkyl dithiocarbamates as generally described in Equation 3.



Where  $R_1, R_2$  are hydrogen, or  $C_1$  to  $C_{60}$  hydrocarbyl.

$M^+$  represents the cationic moiety of dithiocarbamate salt, such as sodium ion ( $Na^+$ ) or potassium ion ( $K^+$ ), triethylammonium ion [ $(C_2H_5)_3N^+H$ ], or other suitable cations such as transition metal ions.

Other epoxides with general structure below are also available for these types of reactions.



Where  $R_3, R_4, R_5$  and  $R_6$  are hydrogen, or  $C_1$  to  $C_{30}$  hydrocarbyl, and optionally can contain additional sulfur, nitrogen and/or oxygen.

Alternatively, halohydrins (such as chlorohydrin) may be used to react with either sodium dialkyl dithiocarbamates or triethylammonium salts of dialkyl dithiocarbamates to form S-hydroxylalkyl N,N-dialkyl dithiocarbamates as generally described in Equation 4.



-continued



Where  $R_7, R_8, R_9$  and  $R_{10}$  are hydrogen, or  $C_1$  to  $C_{60}$  hydrocarbyl,  $R'$  represents the general dithiocarbamate-derived S-hydrocarbyl moiety, and  $X$  is halide (Cl, Br, I).

An excess of one reagent or another can be used. However, the most promising stoichiometry is approximately one mole of dithiocarbamate salts to one mole of halohydrins or epoxides. An excess of up to 5-10 moles of epoxides can on occasion be beneficial. Accordingly, equimolar, less than molar or more than molar quantities of reactants can be used. The reactions of equations (1), (2) or (3) generally take place at temperatures varying from about  $0^\circ$  to  $150^\circ C$ . or at ambient temperature and pressures for periods of time of up to 12 hours or more. Slightly higher pressures may be used if desired.

Subsequently, the S-hydroxylalkyl dihydrocarbyl dithiocarbamates were coborated with hydrocarbyl alcohols in the presence of boronating agents (Equation 5).



and other polymeric structures,

where  $y$  and  $z$  are integers from 0 to 3,  $y+z=3$  and where  $R'$  represents the dithiocarbamate derived S-hydrocarbyl moiety and  $R''$  is  $C_1$  to  $C_{100}$  hydrocarbyl, or sulfur, nitrogen and/or oxygen or boron containing  $C_1$  to  $C_{100}$  hydrocarbyl. One example is that  $R''-OH$  can be an ethoxylated alkyl hydroxy compound (I) or hydroxyesters (II) or (III),



where  $R'''$  is  $C_1$  to  $C_{100}$  hydrocarbyl or sulfur, nitrogen and/or oxygen containing  $C_1$  to  $C_{100}$  hydrocarbyl, and

where  $R_{10}$  is  $C_1$  to  $C_{60}$  hydrocarbyl,  $R_{11}, R_{12}, R_{13}$  and  $R_{14}$  are hydrogen, or  $C_1$  to  $C_{60}$  hydrocarbyl,  $R_{15}$  is  $C_3$  to  $C_{30}$  hydrocarbyl,  $W$  is 1 to 20 and  $V$  is 1 to 6.

When boronating (borating) an excess of one reagent or another can be used. Molar quantities, less than molar quantities or more than molar quantities of a boronating agent can be used. Accordingly, stoichiometric amounts of the boronating agent or up to 100% excess

can be advantageously used. Boric acid, metaborates, trialkyl borates, borate esters, or any other suitable boronating agent may be employed. If a solvent is used the temperature of reaction will vary accordingly. Usually atmospheric or ambient pressure is used, however, higher or lower pressures may be used if desired. The time of reaction for boronating is not critical but will, of course, vary primarily with the temperature and pressure etc. used.

The base lubricants which are useful with the additives of this invention may be any oil of lubricating viscosity, whether natural, i.e., mineral, or synthetic.

The additives may be therefore incorporated into any suitable lubricating media which comprises oils of lubricating viscosity, e.g., mineral or synthetic; or mixtures of mineral and synthetic or greases in which the aforementioned oils are employed as a vehicle or into such functional fluids as hydraulic fluids, brake fluids, power transmission fluids and the like. In general, mineral oils and/or synthetic, employed as the lubricant oil, or grease vehicle may be of any suitable lubricating viscosity range, as for example, from about 45 SSU at 100° F. to about 6000 SSU at 100° F., and, preferably, from about 50 to about 250 SSU at 210° F. These oils may have viscosity indices from about 70 to about 95 preferred. The average molecular weight of these oils may range from about 250 to about 800. Where the lubricant is to be employed in the form of a grease, the lubricating oil is generally employed in an amount sufficient to balance the total grease composition, after accounting for the desired quantity of the thickening agent and other additives components to be included in the grease formulation.

In instances where synthetic oil, or synthetic oils employed as the vehicle for the grease, are desired in preference to mineral oils, or in combination therewith, various compounds of this type may be successfully utilized. Typical synthetic vehicles include polyisobutylene, polybutenes, hydrogenated polydecenes, polypropylene glycol, polyethylene glycol, trimethylolpropane esters, neopentyl and pentaerythritol esters, di(2-ethylhexyl) sebacate, di(2-ethylhexyl) adipate, dibutyl phthalate, fluorocarbons, silicate esters, silanes, esters of phosphorous-containing acids, liquid ureas, ferrocene derivatives, hydrogenated mineral oils, chain-type polyphenyls, siloxanes and silicones (polysiloxanes), alkyl-substituted diphenyl ethers typified by a butyl-substituted bis (p-phenoxy phenyl) ether, phenoxy phenylethers, etc.

Fully formulated lubricating oils may include a variety of additives (for their known purpose) such as dispersants, detergents, inhibitors, antiwear agents, antioxidant, antifoam, pour depressant and other additives including phenates, sulfonates and zinc dithiophosphates. As hereinbefore indicated, the aforementioned additive compounds may be incorporated as multifunctional agents in grease compositions. When high temperature stability is not a requirement of the finished grease, mineral oils having a viscosity of at least 40 SSU at 150° F., and particularly those falling within the range from about 60 SSU to about 6,000 SSU at 100° F. may be employed. The lubricating vehicles of the improved greases of the present invention, containing the above described additives, are combined with a grease forming quantity of a thickening agent. For this purpose, a wide variety of materials dispersed in the lubricating vehicle in grease-forming quantities in such degree as to impart to the resulting grease composition the

desired consistency. Exemplary of the thickening agents that may be employed in the grease formulation are non-soap thickeners, such as surface-modified clays and silicas, aryl ureas, calcium complexes and similar materials. In general, grease thickeners may be employed which do not melt and dissolve when used at the required temperature within a particular environment; soap thickeners such as metallic (lithium or calcium) soaps including hydroxy stearate and/or stearate soaps can be used however, in all other respects, any material which is normally employed for thickening or gelling hydrocarbon fluids or forming greases can be used in preparing the aforementioned improved greases in accordance with the present invention.

Included among the preferred thickening agents are those containing at least a portion of alkali metal, alkaline earth metal or amine soaps of hydroxyl-containing fatty acids, fatty glycerides and fatty esters having from 12 to about 30 carbon atoms per molecule. The metals are typified by sodium, lithium, calcium and barium. Preferred is lithium. Preferred members among these acids and fatty materials are 12-hydroxystearic acid and glycerides containing 12-hydroxystearates, 14-hydroxystearic acid, 16-hydroxystearic acid and 6-hydroxystearic acid.

The entire amount of thickener need not be derived from the aforementioned preferred members significant benefit can be attained using as little thereof as about 15% by weight of the total thickener. A complementary amount, i.e., up to about 85% by weight of a wide variety of thickening agents can be used in the grease of this invention. Included among the other useful thickening agents are alkali and alkaline earth metal soaps of methyl-12-hydroxystearate, diesters of a C<sub>4</sub> to C<sub>12</sub> dicarboxylic acid and tall oil fatty acids. Other alkali or alkaline earth metal fatty acids containing from 12 to 30 carbon atoms and no free hydroxyl may be used. These included soaps of stearic and oleic acids.

Other thickening agents include salt and salt-soap complexes as calcium stearate-acetate (U.S. Pat. No. 2,197,263), barium stearate acetate (U.S. Pat. No. 2,564,561), calcium, stearate-caprylate-acetate complexes (U.S. Pat. No. 2,999,065), calcium caprylate-acetate (U.S. Pat. No. 2,999,066), and calcium salts and soaps of low-, intermediate-and high-molecular weight acids and of nut oil acids.

As has been disclosed hereinabove, the reaction products are useful as multifunctional antioxidant/antiwear/extreme pressure agents. They are added to the lubricating medium in amounts sufficient to impart such properties to the lubricant. More particularly, such properties will be imparted to the lubricant by adding from about 0.01% to about 10% by weight, preferably from about 0.01% to about 3%, of the neat product.

Having described the invention in general terms, the following specific examples are offered for purposes of illustration no intention to limit the invention thereby is to be inferred therefrom.

#### EXAMPLE 1

##### S-2-Hydroxypropyl N,N-di-2-Ethylhexyl Dithiocarbamate

Approximately 483 g (2.0 moles) of bis-2-ethylhexylamine and 204 g (2.02 moles) of triethylamine were mixed together in a two-liter, four-neck reactor equipped with thermometer, dropping funnel, Dean Stark trap, condenser and agitator. Slowly, 160 g (2.1

moles) of carbon disulfide was added dropwise through the dropping funnel at 15°–30° C. over a course of 1.5 hours. Shortly after the completion of carbon disulfide addition, approximately 118 g (2.03 moles) of propylene oxide was slowly added to the reactor at 15°–25° C. over a course of one hour. The reaction exotherm was controlled by using ice-water bath for cooling. It was further stirred for two hours at ambient temperature upon the completion of propylene oxide addition. Thereafter, triethylamine was removed by vacuum distillation at 90°–110° C. The final residue is a viscous, yellowish fluid weighing 748.6 g.

#### EXAMPLE 2

##### S-2-Hydroxypropyl N,N-Dibutyl Dithiocarbamate

Approximately 516 g (4.0 moles) of dibutylamine and 405 g (4.0 moles) of triethylamine were mixed together in a three-liter reactor. Approximately 320 g (4.21 moles) of carbon disulfide was added dropwise to the reactor over a course of three hours. at temperature about 35° C. Upon the completion of carbon disulfide addition, about 235 g (4.045 moles) of propylene oxide was subsequently added over a course of two hours at ambient temperature (about 30° C.). Thereafter, the resulting yellow liquid was stirred temperature for three days under a nitrogen blanket. Finally, triethylamine was vacuum distilled at 100°–110° C. to produce a viscous, reddish liquid as the desired product (1075 g).

#### EXAMPLE 3

##### 2-Ethylhexanol/S-2-Hydroxypropyl N,N-di-2-ethylhexyl Dithiocarbamate Mixed Borates

Approximately 100 g of the above product of Example 1, 50 g of 2-ethyl-1-hexanol, 50 g boric acid, and 100 g toluene were mixed together in a one-liter, four-neck reactor equipped with thermometer, N<sub>2</sub> sparget, Dean Stark trap condenser and agitator. This mixture was heated at 80°–85° C. for two hours, and then the reaction temperature was gradually increased up to boiling toluene at 112°±2° C. over a course of three hours. A catalytic amount of Sag 47 defoamant was added to reduce the formation of foaming material, and about 150 g mineral oil diluent was added for easy handling. A total amount of 21.4 ml of water was collected in the Dean Stark trap.

An additional hour of heating produced no more water of reaction. The toluene was subsequently removed by distillation to produce a dark brownish fluid as desired product.

#### EXAMPLE 4

##### 2-Butanol/S-2-Hydroxypropyl N,N-Dibutyl Dithiocarbamate Mixed Borates

Approximately 100 g of the above product of Example 2, 50 g of 2-butanol, 50 g boric acid, and 100 g toluene were reacted at 80°–115° C. over a course of six hours. A total amount of 29 ml of water was collected in the Dean Stark trap. The volatiles were vacuum distilled until water evolution ceased. The final product was a viscous, yellow fluid.

The mixed borates (Examples 3 and 4) were blended into fully formulated mineral oils and evaluated for antioxidant performance by Method M334-2, Catalytic Oxidation Test at 325° F. for 40 hours (Table 1); Method M334-3, Cataytic Oxidation Test at 325° F. for 72 hours (Table 2).

The Catalytic Oxidation Test may be summarized as follows.

The test lubricant composition is subjected to a stream of air which is bubbled through the composition at a rate of 5 liters per hour. Present in the composition are metals commonly used as materials of engine construction, namely:

- (a) 15.6 sq. in. of sand-blasted iron wire,
- (b) 0.78 sq. in. of polished copper wire,
- (c) 0.87 sq. in. of polished aluminum wire, and
- (d) 0.167 sq. in. of polished lead surface.

Inhibitors for oil are rated on the basis of prevention of oil deterioration as measured by the increase in acid formation or neutralization number (NN) and kinematic viscosity (KV) occasioned by the oxidation.

TABLE 1

| Item                                                                  | Additive Conc. (wt %) | Percent Change        |                         |           | Lead Loss |
|-----------------------------------------------------------------------|-----------------------|-----------------------|-------------------------|-----------|-----------|
|                                                                       |                       | Viscosity $\Delta$ KV | Acid Number $\Delta$ NN | Lead Loss |           |
| Base Oil (200 second solvent refined paraffinic neutral, mineral oil) | —                     | 57.9                  | 4.78                    | 2.9       |           |
| Example 3                                                             | 1.0                   | 13.6                  | 2.10                    | 0.2       |           |
| Example 4                                                             | 1.0                   | 5.1                   | 0.08                    | 0.4       |           |

TABLE 2

| Item                                                                  | Additive Conc. (wt %) | Percent Change        |                         |           | Lead Loss |
|-----------------------------------------------------------------------|-----------------------|-----------------------|-------------------------|-----------|-----------|
|                                                                       |                       | Viscosity $\Delta$ KV | Acid Number $\Delta$ NN | Lead Loss |           |
| Base Oil (200 second solvent refined paraffinic neutral, mineral oil) | —                     | 99.4                  | 8.53                    | 5.2       |           |
| Example 4                                                             | 1.0                   | 12.1                  | 0.30                    | 0.0       |           |

As shown above, the products of this invention show very good antioxidant activity as evidenced by control of increase in acidity, viscosity and lead loss.

The dithiocarbamate-derived borates were also evaluated for antiwear performance using the Four-Ball Test (Table 3).

The Four Ball Wear Test, for example, disclosed in U.S. Pat. No. 3,423,316. In general, in this test three steel balls of SAE 52100 steel are held in a ball cup. A fourth ball positioned on a rotatable vertical axis is brought into contact with the three balls and is rotated against them. The force with which the fourth is held against the three stationary balls may be varied according to a desired load. The test lubricant is added to the ball cup and acts as a lubricant for the rotation. At the end of the test, the steel balls are investigated for wear scars; the extent of scarring represents the effectiveness of the lubricant as an antiwear agent. Results are also reported as wear rates in volume of wear per unit sliding distance per kilogram load. The lower the wear rate, the more effective the lubricant as an antiwear agent.

TABLE 3

Four Ball Test

| Item                              | Wear Scar Diameter in MM<br>(60 Kg Load, 30 Minute,<br>2000 rpm and 200° F.) |  |
|-----------------------------------|------------------------------------------------------------------------------|--|
|                                   |                                                                              |  |
| Base Oil (80%                     | 4.37                                                                         |  |
| Solvent Paraffinic                |                                                                              |  |
| Bright, 20% Solvent               |                                                                              |  |
| Paraffinic Neutral                |                                                                              |  |
| Minerals Oils)                    |                                                                              |  |
| 1% Example 3<br>in above Base Oil | 0.96                                                                         |  |
| 1% Example 4<br>in above Base Oil | 1.12                                                                         |  |

As can be seen from the above wear test results, the products described exhibit considerable antiwear activity.

The dithiocarbamate-derived borates were also evaluated for copper corrosion characteristics (Table 3). The Copper Corrosion Test employed for this purpose was a standard ASTM Test D-130 which, in general, comprises immersion of a polished copper strip in the material to be tested for a period of 3 hours at a temperature of 250° F. At the end of this period the copper strip is removed, washed, and rated for degree of corrosion by comparison with the ASTM standard strips. Test data is reported in Table 3. The concentration of the respective examples is in Wt. % in 200" SPN, i.e., 200 second solvent paraffinic neutral.

TABLE 4

Copper Strip Corrosivity (250° F., 3 Hours)

| Item                                                                          | Additive<br>Conc. (wt %) | Corrosivity<br>Rating |
|-------------------------------------------------------------------------------|--------------------------|-----------------------|
| Base Oil (200 Second,<br>Solvent Refined, Paraffinic<br>Neutral, Mineral Oil) | —                        | 1A                    |
| Example 3                                                                     | 1.0                      | 1A                    |
| Example 4                                                                     | 1.0                      | 1A                    |

As shown above, the products of this invention show very good antioxidant activity as evidenced by control of increase in acidity and viscosity, and the products are non-corrosive to copper metal.

The use of additive concentrations of mixed alcohol/-dithiocarbamate-derived hydroxy borates in premium quality automotive and industrial lubricants will significantly enhance the stability, reduce the wear, and extend the service life. These novel compositions described in this application are useful at low concentrations and do not contain any potentially undesirable metals, phosphorus, or chloride, and do not cause any corrosivity problem. These multifunctional antioxidant/-antiwear additives can be commercially made using an economically favorable process which can be readily implemented using known technology in existing equipment.

Although the present invention has been described with preferred embodiments, it is to be understood that modifications and variations may be resorted to, without departing from the spirit and scope of this invention, as those skilled in the art will readily understand. Such modifications and variations are considered to be within the purview and scope of the appended claims.

What is claimed is:

1. A lubricant composition comprising a major amount of a lubricating oil or grease and a minor amount of a multifunctional antioxidant antiwear, ex-

treme pressure borated dihydrocarbyl dithiocarbamate reaction product having the structural formula:



where R' is the dithiocarbamate, R'' is C<sub>1</sub> To C<sub>100</sub> hydrocarbyl, said hydrocarbyl group optionally containing at least one heteroatom selected from a member of the group consisting of sulfur, nitrogen, oxygen or boron, y + z are integers and the sum of y + z = 3, prepared by (1) reacting an alkali metal hydroxide or trihydrocarbyl amine, a dihydrocarbyl amine and carbon disulfide wherein said first step comprises the reaction having the structural formulas:



or



where R<sub>1</sub> and R<sub>2</sub> are C<sub>1</sub> to about C<sub>60</sub> hydrocarbyl and R<sub>3</sub> is C<sub>1</sub> to about C<sub>50</sub> hydrocarbyl and M is a metal cation and (2) reacting the product of (1) with a hydrocarbyl oxide thereby forming S-hydroxyhydrocarbyl dihydrocarbyl dithiocarbamates wherein said second step comprises the reaction structural formulas:



where R<sub>1</sub>, R<sub>2</sub> are C<sub>1</sub> to C<sub>60</sub> hydrocarbyl, where R<sub>3</sub>, R<sub>4</sub>, R<sub>5</sub> and R<sub>6</sub> are hydrogen or C<sub>1</sub> to about C<sub>30</sub> hydrocarbyl optionally containing sulfur, nitrogen and/or oxygen, R<sub>7</sub> is the hydrocarbyl moiety derived from said oxide and where M<sup>+</sup> is the cationic moiety of a dithiocarbamate salt and (3) thereafter coborating the product of (2) with a C<sub>1</sub>-C<sub>100</sub> hydrocarbyl alcohol in the presence of a borating agent wherein the reaction temperatures vary from 0° to about 150° C., the molar ratios of reactants vary from equimolar to less than molar to more than molar under ambient pressures.

2. The composition of claim 1 wherein the borating agent is selected from the group consisting of boric acid, metaborates, or trialkyl borates.

3. The composition of claim 2 wherein the borating agent is boric acid.

4. The composition of claim 2 wherein said reaction product is 2-ethylhexanol/S-2-hydroxypropyl N,N-di-2-ethylhexyl dithiocarbamate borate.

5. The composition of claim 2 wherein said reaction product is 2-butanol/S-2-hydroxypropyl N,N-dibutyl dithiocarbamate borate.

6. The lubricant composition of claim 1 wherein the lubricating oil is selected from the group consisting of (1) mineral oils, (2) synthetic oils, (3) mixtures of mineral and synthetic oils or (4) a grease prepared from (1), (2) or (3).

7. The lubricant composition of claim 6 wherein the oil is (1) a mineral oil.

8. The lubricant composition of claim 6 wherein the oil is (2) a synthetic oil.

9. The lubricant composition of claim 6 wherein the oil is (3) a mixture of mineral and synthetic oils.

10. The lubricant composition of claim 6 wherein said composition is (4) a grease.

11. The lubricant composition of claim 6 comprising from about 0.01 to about 10 wt % of said borated reaction product.

12. The composition of claim 11 comprising from about 0.01 wt % to about 3 wt % of said borated reaction product.

13. A process of preparing a borated dihydrocarbyl dithiocarbamate reaction product having the structural formula:



where R' is the dithiocarbamate, R'' is C<sub>1</sub> to C<sub>100</sub> hydrocarbyl, said hydrocarbyl group optionally containing at least one heteroatom selected from a member of the group consisting of sulfur, nitrogen, oxygen or boron, y+z are integers and the sum of y+z=3, comprising (1) reacting an alkali metal hydroxide or a trihydrocarbyl amine, a dihydrocarbylamine and carbon disulfide in non-aqueous media wherein said first step comprises the reaction having the structural formulas:



55

where R<sub>1</sub> and R<sub>2</sub> are C<sub>1</sub> to about C<sub>60</sub> hydrocarbyl and R<sub>3</sub> is C<sub>1</sub> to about C<sub>50</sub> hydrocarbyl and M is a metal cation and (2) reacting the product of (1) with a hydrocarbyl oxide to form a hydroxyhydrocarbyl N,N-dihydrocarbyl dithiocarbamate wherein said second step comprises the reaction structural formulas:



where R<sub>1</sub>, R<sub>2</sub> are C<sub>1</sub> to C<sub>60</sub> hydrocarbyl, where R<sub>3</sub>, R<sub>4</sub>, R<sub>5</sub> and R<sub>6</sub> are hydrogen or C<sub>1</sub> to about C<sub>30</sub> hydrocarbyl optionally containing sulfur, nitrogen and/or oxygen, R<sub>7</sub> is the hydrocarbyl moiety derived from said oxide and where M<sup>+</sup> is the cationic moiety of a dithiocarbamate salt and (3) thereafter coborating the resultant product of (2) with C<sub>1</sub>-C<sub>100</sub> hydrocarbyl alcohol in the presence of a borating agent wherein the reaction temperatures vary from 0° to about 150° C., the molar ratios of reactants vary from equimolar to less than molar to more than molar under ambient pressure.

25 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9